

## 1

3,249,439

**POLYHYDROXYETHER PHOTOGRAPHIC FILMS**  
 Thomas E. Bugel, New Market, N.J., assignor to Union Carbide Corporation, a corporation of New York  
 No Drawing. Continuation of application Ser. No. 90,923, Feb. 23, 1961. This application Nov. 25, 1964, Ser. No. 414,001  
 14 Claims. (Cl. 96—87)

This is a continuation of application Serial No. 90,923, filed February 23, 1961, now abandoned.

This invention relates to photographic films having improved dimensional stability and freedom from curl. More particularly, the invention relates to a novel film support for photographic films which confers improvements in dimensional stability and curl resistance to photographic film structures.

Photographic film comprises: a film support, generally glass, paper or polymeric film; a photosensitive "emulsion" containing one or more silver halides suspended in gelatin; and usually an intermediate gelatin layer generally termed "subbing" to insure adhesion of the emulsion to the film support.

The most widely adopted film supports for photosensitive emulsions are those of organic esters of cellulose, e.g., cellulose nitrate and cellulose triacetate. Few other materials are useful as film supports for photosensitive emulsions. Specialty film supports include polyethylene terephthalate, polystyrene and polycarbonate, but their

10 5 It has now been discovered that these and other objects are achieved with a photographic film comprising a photosensitive emulsion adhered to a poly(hydroxyether) film support either through an intermediate layer of gelatin subbing or directly. The poly(hydroxyether) film supported photographic film is superior to photographic films heretofore made in:

(1) *Adherence of the gelatin to the film support.*—Poly(hydroxyether) film support outperforms polyethylene terephthalate, polystyrene and polycarbonate film supports in resistance to delaminating during development of the latent image; or

(2) *Resistance to curl and dimensional stability.*—Poly(hydroxyether) film support is unaffected by a coating of gelatin subbing; but cellulose triacetate film quickly rolls into a tight curl after coating with gelatin subbing. Poly(hydroxyether) is unaffected by short or long exposures to developing solutions; but cellulose triacetate is adversely affected by long exposures to developing solutions and even short term exposure (2 minutes) to a gelatin subbing formulation.

20 15 25 30 A tabular comparison of the performance in typical developing solutions of poly(hydroxyether) film support in comparison to cellulose triacetate film support is presented in Table I below.

Table I

RESISTANCE TO CURL—POLY(HYDROXYETHER) (PHE) VS. CELLULOSE TRIACETATE (CTA)

|                                                                                                                            | After Two Minutes                                |                                                  | After 48 Hours 0                                 |                                                                  |
|----------------------------------------------------------------------------------------------------------------------------|--------------------------------------------------|--------------------------------------------------|--------------------------------------------------|------------------------------------------------------------------|
|                                                                                                                            | PHE<br>(0.003" thick)                            | CTA<br>(0.003" thick)                            | PHE<br>(0.003" thick)                            | CTA<br>(0.003" thick)                                            |
| (1) Control—68° F. 50% Relative Humidity                                                                                   | Flat, glossy                                     | Flat, glossy                                     | Flat, glossy                                     | Flat, glossy                                                     |
| (2) Immersion in Developer (before water dilution)                                                                         | Flat, glossy but<br>spotted from<br>dried salts. | Flat, glossy but<br>spotted from<br>dried salts. | Flat, glossy but<br>spotted from<br>dried salts. | Spotted and curled<br>and wrinkled un-<br>evenly. Yel-<br>lowed. |
| (3) Immersion in Acid Stop Bath                                                                                            | Flat, glossy                                     | Flat, glossy                                     | Flat, glossy                                     | Curled along edges.<br>Do.                                       |
| (4) Immersion in Fixing Bath                                                                                               | Flat, glossy but<br>spotted.                     | Flat, glossy but<br>spotted.                     | Warp and curled<br>unevenly<br>throughout.       | Do.                                                              |
| (5) Immersion in Gelatin "Subbing" (Gelatin,<br>10 g.; Glacial Acetic Acid, 50 cc.; Water, 50 cc.;<br>Methanol, 1,000 cc.) | Flat, glossy                                     | Do                                               | Do                                               | Do                                                               |

use is not widespread because gelatin containing compositions can be adhered only with difficulty to these film supports.

Cellulose triacetate is the most popular flexible film support, for roll film and movie film. This material, however, exhibits the usual undesirable properties of cellulose esters, particularly a pronounced tendency to absorb moisture. Cellulose triacetate absorbs 3.5% of its own weight in water in a 70° F. environment with 90% of relative humidity (R.H.). Also, cellulose triacetate film is inherently brittle and must be highly plasticized, e.g., with from 5 to 25% triphenyl phosphate. Presence of plasticizers means weight loss, thermal brittleness and dimensional instability upon film support aging, especially at elevated temperatures. As is typical of cellulose ester films, cellulose triacetate curls badly upon immersion in water or photographic solutions unless the film is modified during manufacture by costly and laborious techniques.

It is an object, therefore, of the present invention to provide a photographic film which is improved in resistance to water absorption and dimensionally stable and in which the gelatin of the emulsion or subbing adheres

55 60 65 The superiority of poly(hydroxyether) film support to cellulose triacetate film support in dimensional stability is shown in Table II following. Tests were conducted with various combinations of temperature and relative humidity. Film support samples 20" x 1" x 0.007" were placed in these environments for periods of from 24 to 120 hours. The difference in the long dimension before and after the test is reported as percent change. A plus (+) indicates an increase in the long dimension, and conversely a minus (—) indicates a decrease.

Also given in Table II are the results of maintaining film support samples of poly(hydroxyether) and cellulose triacetate at 177° F. for 24 hours. The weight loss is reported as percent of original weight.

70 75 Also given in Table II are the results of thermal brittleness tests on a 0.003 inch thick section of both poly(hydroxyether) film support and cellulose triacetate. After aging for the indicated period the samples were folded and unfolded by hand. The number of times the film support could be folded on itself before the film split is reported in Table II. In the case of aged cellulose triacetate cracks appeared well before splitting occurred, as indicated in Table II. In all cases the poly(hydroxyether)

## 2

tenaciously to the film support before, during and after developing.

It is another object to provide method for rapidly and simply making photographic film without use of a subbing layer.

It has now been discovered that these and other objects are achieved with a photographic film comprising a photosensitive emulsion adhered to a poly(hydroxyether) film support either through an intermediate layer of gelatin subbing or directly. The poly(hydroxyether) film supported photographic film is superior to photographic films heretofore made in:

(1) *Adherence of the gelatin to the film support.*—Poly(hydroxyether) film support outperforms polyethylene terephthalate, polystyrene and polycarbonate film supports in resistance to delaminating during development of the latent image; or

(2) *Resistance to curl and dimensional stability.*—Poly(hydroxyether) film support is unaffected by a coating of gelatin subbing; but cellulose triacetate film quickly rolls into a tight curl after coating with gelatin subbing. Poly(hydroxyether) is unaffected by short or long exposures to developing solutions; but cellulose triacetate is adversely affected by long exposures to developing solutions and even short term exposure (2 minutes) to a gelatin subbing formulation.

A tabular comparison of the performance in typical developing solutions of poly(hydroxyether) film support in comparison to cellulose triacetate film support is presented in Table I below.

film support outperformed the cellulose triacetate by a wide margin.

there are substituents exclusive of the hydroxyl groups on either or both of the aromatic divalent hydrocarbon

Table II

## PHYSICAL AND DIMENSIONAL STABILITY POLY(HYDROXYETHER) VS. CELLULOSE TRIACETATE

| Environment                            | Measured Effect                                                       | Observed Change:<br>Cellulose<br>Triacetate | Poly<br>(hydroxy-<br>ether) |
|----------------------------------------|-----------------------------------------------------------------------|---------------------------------------------|-----------------------------|
| 150° F., 90% Relative Humidity.        | Dimensional Change:<br>24 hrs.-----<br>48 hrs.-----<br>120 hrs.-----  | -0.20%<br>-0.40%<br>-0.90%                  | 0.0%<br>+0.1%<br>-0.1%      |
| 150° F. Dry Air <5% Relative Humidity. | Dimensional Change:<br>24 hrs.-----<br>48 hrs.-----<br>120 hrs.-----  | -0.4%<br>-0.5%<br>-0.8%                     | -0.1%<br>-0.2%<br>-0.2%     |
| 177° F. Dry Air <5% Relative Humidity. | Weight Loss, 24 hrs.-----                                             | 2.9%                                        | 0.1%                        |
| Do-----                                | Thermal Embrittlement:<br>0 hrs.-----<br>24 hrs.-----<br>72 hrs.----- | 42<br>131<br>216                            | 50<br>21<br>19              |

<sup>1</sup> Cracks at 20.

2 Cracks at 3-5.

The poly(hydroxyether) film supports of the present invention are prepared by extrusion, casting from solution, or calendering a film-forming poly(hydroxyether) resin. These resins are reaction products of a dihydric polynuclear phenol and an epitriolhydrin in about equimolar amounts such as are prepared in accordance with U.S. Patent 2,602,075, issued July 1, 1952, to A. S. Carpenter et al., which is herewith incorporated by reference. 25 30

The film-forming poly(hydroxyethers) have reduced viscosities of from about 0.3 to 1.2 and preferably from 0.43 to 0.65 measured as a 0.2 gram sample in 100 milliliters of tetrahydrofuran at 25° C.

The poly(hydroxyethers) contain as the recurring units a residue of a dihydric polynuclear phenol having the general formula  $-\text{O}-\text{E}-\text{O}-$  wherein E is the nucleus of the dihydric polynuclear phenol in which the hydroxyl groups are attached to different nuclei and a group having the general formula



wherein R and R<sup>1</sup> which can be the same or different are hydrogen or methyl, with the recurring units having the general formula



$E$ ,  $R$  and  $R^1$  being as previously defined.

Illustrative of dihydric polynuclear phenols which can be reacted with epihalohydrins to produce the thermoplastic poly(hydroxyethers) of the present invention are the dihydric polynuclear phenols having the general formula



wherein Ar is an aromatic divalent hydrocarbon radical such as naphthylene and phenylene with phenylene being preferred for purposes of this invention; Y and Y<sub>1</sub>, which can be the same or different, are alkyl radicals such as methyl, n-propyl, n-butyl, n-hexyl, n-octyl and the like, preferably alkyl radicals having a maximum of 4 carbon atoms; or halogen atoms, i.e., chlorine, bromine, iodine, or fluorine; or alkoxy radicals such as methoxy, methoxymethyl, ethoxy, ethoxyethyl, n-butoxy, amyloxy and the like, preferably an alkoxy radical having a maximum of 4 carbon atoms. It is to be understood that whenever

groups, these substituents can be the same or different;  $m$  and  $z$  are integers having a value of from 0 to a maximum value corresponding to the number of hydrogen atoms on the aromatic ring (Ar) which can be replaced by substituents and can have the same or different values; and  $R_1$  is a divalent radical, as for example



or  $-O-$ , or  $-S-$ , or  $-SO-$ , or  $-SO_2-$ , or  $-S-S-$ , or a divalent hydrocarbon radical as, for example, an alkylene radical such as methylene, ethylene, trimethylene, tetramethylene, pentamethylene, hexamethylene, 2-ethyl hexamethylene, octamethylene, nonamethylene, decamethylene, and the like; an alkylidene radical such as ethylidene, propylidene, isopropylidene, isobutylidene, amylidene, isoamylidene, 1-phenyl ethylidene and the like, or a cycloaliphatic radical, such as 1,4-cyclohexylene, 1,3-cyclohexylene, cyclohexylidene, and the like, or halogenated alkylidene, alkylene or cycloaliphatic radicals, alkoxy and aryloxy substituted alkylidene, alkylene or cycloaliphatic radicals such as methoxy methylene, ethoxy methylene, ethoxy ethylene, 2-ethoxy trimethylene, 3-ethoxy pentamethylene, 1,4 - (2-methoxycyclohexane), phenoxy ethylene, 2-phenoxy trimethylene, 1,3-(2-phenoxy cyclohexane) and the like, aralkylene radicals, such as phenyl ethylene, 2-phenyl trimethylene, 1-phenyl pentamethylene, 2-phenyl decamethylene, and the like, aromatic radicals, such as phenylene, naphthylene, and the like, halogenated aromatic radicals, such as 1,4-(2-chlorophenylene), 1,4 - (2 - bromophenylene), 1,4-(2-fluorophenylene), and the like; alkoxy and aryloxy substituted aromatic radicals, such as 1,4-(2-methoxyphenylene), 1,4 - (2-ethoxyphenylene), 1,4-(2-n-propoxyphe nylene), 1,4-(2-phenoxyphenylene), and the like, alkyl substituted aromatic radicals, such as 1,4-(2-methylphenylene), 1,4-(2-ethylphenylene), 1,4-(2-n-propylphenylene), 1,4-(2-n-butylphenylene), 1,4-(2-n-dodecylphenylene) and the like; or  $R_1$  can be a ring which is fused to one of the Ar groups as is the case, for example, in the compound having the formula:



0

0

or  $R_1$  can be a polyalkoxy radical such as polyethoxy, polypropoxy, polythioethoxy, polybutoxy, polyphenylethoxy; or  $R_1$  can be a radical containing a silicon atom as, for example, polydimethylsiloxy, polydiphenylsiloxy, polymethylphenylsiloxy and the like; or  $R_1$  can be two or more alkylene or alkylidene radicals separated by an aromatic ring, a tertiary amino group, an ether linkage, a carbonyl group or separated by a linkage containing sulfur such as sulfur, sulfoxide and the like.

Particularly preferred are the dihydric polynuclear phenols having the general formula:



wherein  $Y$ ,  $Y_1$  are as previously defined,  $m$  and  $z$  have values from 0 to 4 inclusive and  $R_1$  is an alkylene or alkylidene group, preferably having from 1 to 3 carbon atoms inclusive or  $R_1$  is a saturated group having the formula:



or



Poly(hydroxyethers) produced using the dihydric polynuclear phenols described in the preceding paragraph have extremely good mechanical properties. In addition poly(hydroxyethers) produced using a dihydric polynuclear phenol wherein  $R_1$  is a saturated group having the formula



or



have heat distortion temperatures which are relatively high.

Exemplary of other specific dihydric phenols include among others the

Bis-(hydroxyphenyl)-alkanes such as

2,2-bis-(p-hydroxyphenyl)-propane, commonly referred to as bisphenol-A;

2,4'-dihydroxydiphenylmethane,

Bis-(2-hydroxyphenyl)-methane,

Bis-(4-hydroxyphenyl)-methane,

Bis-(4-hydroxy-2,6-dimethyl-3-methoxyphenyl)-methane,

1,1-bis-(4-hydroxyphenyl)-ethane,

1,2-bis-(4-hydroxyphenyl)-ethane,

1,1-bis-(4-hydroxy-2-chlorophenyl)-ethane,

1,1-bis-(3,5-dimethyl-4-hydroxyphenyl)-ethane,

1,3-bis(3-methyl-4-hydroxyphenyl)-propane,

2,2-bis-(3-phenyl-4-hydroxyphenyl)-propane,

2,2-bis-(3-isopropyl-4-hydroxyphenyl)-propane,

2,2-bis-(2-isopropyl-4-hydroxyphenyl)-propane,

2,2-bis-(4-hydroxynaphthyl)-propane,

2,2-bis-(4-hydroxyphenyl)-pentane,

3,3-bis-(4-hydroxyphenyl)-pentane,

2,2-bis-(4-hydroxyphenyl)-heptane,

Bis-(4-hydroxyphenyl)-phenylmethane,

Bis-(4-hydroxyphenyl)-cyclohexylmethane,

1,2-bis-(4-hydroxyphenyl)-1,2-bis-(phenyl)-propane,

2,2-bis-(4-hydroxyphenyl)-1-phenylpropane and the like;

Dihydroxy biphenyls such as 4,4'-dihydroxybiphenyl,

2,2'-dihydroxybiphenyl, 2,4'-dihydroxybiphenyl and the like;

Di(hydroxyphenyl)sulfones such as bis(4-hydroxyphenyl)-sulfone,

2,4'-dihydroxydiphenyl sulfone,

5'-chloro-2,4'-dihydroxydiphenyl sulfone,

5'-chloro-4,4'-dihydroxydiphenyl sulfone,

3'-chloro-4,4'-dihydroxydiphenyl sulfone and the like;

Di(hydroxyphenyl) ethers such as bis-(4-hydroxyphenyl)-ether, the 4,3'-, 4,2'-, 2,2'-, 2,3'-dihydroxy-diphenyl

ethers, 4,4'-dihydroxy-2,6-dimethyldiphenyl ether, bis-(4-hydroxy-3-isobutylphenyl)-ether, bis-(4-hydroxy-3-isopropylphenyl)-ether, bis-(4-hydroxy-3-chlorophenyl)-ether, bis-(4-hydroxy-3-fluorophenyl)-ether,

bis-(4-hydroxy-3-bromophenyl)-ether, bis-(4-hydroxy-3-chloronaphthyl)-

ether, bis-(2-hydroxybiphenyl)-ether, 4,4'-dihydroxy-2,6-dimethoxy-diphenyl ether, 4,4'-dihydroxy-2,5-diethoxydiphenyl ether, and the like;

Also suitable are 1,1-bis-(4-hydroxyphenyl)-2-phenyl-

ethane, 1,3,3-trimethyl-1-(4-hydroxyphenyl)-6-

hydroxyindane, 2,4-bis-(p-hydroxyphenyl)-4-methyl-

pentane and the like.

Mixtures of dihydric polynuclear phenols can also be employed and wherever the term "dihydric polynuclear phenol" is used herein, mixtures of these compounds are intended to be included.

Among suitable epihalohydrins and mixtures thereof which can be reacted with dihydric polynuclear phenols to produce the thermoplastic poly(hydroxyethers) of this invention are those having the general formula



wherein  $R$  and  $R^1$  which can be the same or different are hydrogen or methyl and  $X$  is a halogen atom, i.e., chlorine, bromine, and the like. Specific epihalohydrins are epichlorohydrin, epibromohydrin, 1,2-epoxy-1-methyl-

3-chloropropane and 1,2-epoxy-2-methyl-3-chloropropane.

To prepare a photographic film using the poly(hydroxyether) film support, in a preferred manner, a clear film is cast from solution, suitably from a solution in

tetrahydrofuran, dioxane, chloroform, dimethylformamide, Cellosolve or diacetone dialcohol, onto a glass plate or similar substrate, or extruded at the desired thickness. Film supports of poly(hydroxyether) are suitably of from 0.001 to 0.010 inch in thickness, with thickness of

0.003 to 0.07 being preferred for best combination of body and flexibility.

To the poly(hydroxyether) film support there can be applied a subbing, generally a gelatin based composition, prior to application of the photosensitive emulsion.

Surprisingly, we have discovered that the poly(hydroxyether) film supports described herein are uniquely advantageous in their wettability with photosensitive gelatin emulsion. This property permits use of a special photosensitive emulsion which contains a water-soluble poly-

(hydroxyether) solvent, e.g., tetrahydrofuran, dioxane, dimethylformamide, Cellosolve and diacetone dialcohol, and can be applied directly to the film support without use of an intermediate layer of subbing. The use of this technique is illustrated in Examples 3, 4, 6, 8 and 10 hereof.

Typically the photosensitive emulsion is prepared by slowly adding a dilute solution of silver nitrate with vigorous stirring to a solution of gelatin and potassium chloride, iodide or bromide. Exceedingly fine silver halide crystals are thereby formed. The emulsion or, more properly, the suspension, of silver halide in the gelatin is "ripened" to make it more sensitive to light. Ripening is accomplished by maintaining the emulsion at an elevated temperature, e.g., 90° F. for several hours. After ripening the gelatin solution is cooled to a stiff mass which is shredded to "noodles." The noodles are washed to free the emulsion of undesired salts, e.g., potassium salts. After washing, the noodles are melted and kept heated for a time to further sensitize the emulsion, then additives, such as hardening agents, solvents for the film support and sensitizers are incorporated. The emulsion is then coated onto the subbing on the film support or, if a water soluble solvent for poly(hydroxyether) such as are listed above was incorporated into the emulsion, directly onto the poly(hydroxyether) film support.

Exposing the film to a light source causes an invisible "latent image" in the emulsion where the silver halides have been exposed to light. To change the invisible latent image to a visible image, a developing agent is used. Developing agents comprise:

(1) A solvent to swell the gelatin of the emulsion and permit the developer to reach the silver halide crystals;

(2) A developer, i.e., a compound which is capable of changing exposed silver halide crystals to metallic silver without any effect on unexposed silver halide crystals. Typical chemicals which can reduce AgCl, AgI and AgBr to elemental Ag are hydroquinone, p-aminophenol, p-phenylenediamine and the like. Where colored images are desired a plurality, e.g., three, layers of silver halide emulsion are used on the film support, and the developer is used with a "coupler" e.g., dimethyl-p-phenylenediamine,  $\alpha$ -naphthol, indophenol blue, chloro- $\alpha$ -naphthol, 4-amino-N-ethyl - N - ( $\beta$ -methanesulfonamidoethyl) - m-toluidine sesquisulfate monohydrate and the like, either embedded in the emulsion or present in the developing agent;

(3) A preservative such as  $\text{Na}_2\text{SO}_3$  which combines chemically with oxidation products formed in the developing agent and so keeps the developer clear;

(4) An activator such as sodium hydroxide, sodium carbonate or borax which by alteration of the pH of the developing agent varies the activity of the developer; and

(5) A restrainer, e.g., potassium bromide, to inhibit "fog" formation (metallic silver produced by action of the developer on unexposed silver halide).

Most commercial developing agents for silver halide photographic emulsion contain such ingredients. The developing agents are not critical to this invention, however, and any combination of ingredients capable of producing visible images from photosensitive emulsion layers can be employed.

When the emulsion has been sufficiently developed the development reaction is stopped either by use of running rinse water or by use of an acid rinse, a "stop-bath" such as acetic acid, which neutralizes the activator in the emulsion layer.

When the developing reaction has been stopped the unexposed silver halides are removed from the emulsion by a "fixing bath" which is a water solution of a compound which forms complexes with silver ions, e.g., sodium thiosulfate or ammonium thiosulfate. The fixing bath may contain acids, preservatives, hardeners, buffers and the like in order to fix the image and prevent further light sensitivity.

The following examples are illustrative of this invention. All parts and percentages are by weight.

#### EXAMPLE 1

A photosensitive film was prepared by dip-coating a 0.003 inch thick uncoated film support of an extruded

5 poly-(hydroxyether) having a reduced viscosity of 0.46 measured as a 0.2 gram sample in 100 milliliters of tetrahydrofuran and the recurring unit



10 with a photosensitive composition in solution comprising

|                         |    |      |
|-------------------------|----|------|
| Water                   | cc | 1000 |
| Ferric ammonium citrate | g  | 90   |
| Tartaric acid           | g  | 15   |
| Silver nitrate          | g  | 37.5 |
| Disodium sulfosuccinate | g  | 11.4 |

15 The dip-coated poly(hydroxyether) film support was air dried in complete darkness. The coating was exposed to light through a stencil. A transparency with a sharp brown image was obtained.

20 Example 1 is illustrative of the use of poly(hydroxyether) as film support in applications where a gelatin emulsion of silver halides is not used to produce an image. Other useful image producing compositions readily adhere to the poly(hydroxyether) film support. For example, there can be applied to the film supports of this invention (1) "dichromate process" photosensitive coatings, e.g., potassium dichromate in glues, gums or gelatins wherein exposure to light causes selective hardening of the gelatin, gum or glue to produce an image; the inclusion of carbon black in the dichromate process coatings (the "Carbon Process") provides black images; (2) "diazoy process" coatings which upon exposure to light and treatment with alkali and phenolic compounds produce images by appearance of selectively formed dyes; and (3) blueprint process coatings where ferric salts are adhered to the film support and reduced to ferrous salts to produce an image, or where platinum and palladium salts are used for the same purpose and effect.

25 It is seen, therefore, that the present invention is not limited to use of poly(hydroxyether) as film supports for gelatin emulsions of silver halides but rather extends to use of any photosensitive coating on poly(hydroxyether) film supports.

#### EXAMPLE 2

30 A photographic film was prepared by first applying to the face of an extruded 0.003 inch thick film support of the same poly(hydroxyether) as used in Example 1, a subbing comprising

|                       |    |      |
|-----------------------|----|------|
| Gelatin               | g  | 10   |
| Acetic acid (glacial) | cc | 50   |
| Water                 | cc | 50   |
| Methanol              | cc | 1000 |

35 and air drying. Then a photosensitive emulsion prepared in darkness using

|                                                                                            |    |      |
|--------------------------------------------------------------------------------------------|----|------|
| (1) Mixed silver halides (dehydrated emulsion)                                             | g  | 150  |
| Dissolved in water                                                                         | cc | 2170 |
| (2) Saponin                                                                                | g  | 3    |
| Dissolved in water                                                                         | cc | 97   |
| (3) Methanol                                                                               | cc | 100  |
| (4) Ammonium chrome alum                                                                   | g  | 1.2  |
| $(\text{Cr}_2(\text{SO}_4)_3 \cdot (\text{NH}_4)_2\text{SO}_4 \cdot 24\text{H}_2\text{O})$ | cc | 9    |
| Dissolved in water                                                                         | cc |      |

40 45 50 55 60 65 was applied in darkness to the subbing layer on the poly (hydroxyether) film support and the assembly air dried.

The photographic film was exposed to light through a negative. Developing, fixing and washing was by standard techniques using standard developers, stop baths and fixing baths. A clear reverse image of the negative was obtained.

Control 2A.—The procedure of Example 2 was followed but using a 0.003 inch thick sheet of cellulose triacetate as film support. The photosensitive emulsion and

the subbing layer lifted off the film support in the developer solution.

**Control 2B.**—The procedure of Example 2 was followed but using a 0.003 inch thick sheet of polycarbonate as film support. The photosensitive emulsion and the subbing layer lifted off the film support in the developer solution.

### EXAMPLE 3

A photographic film was prepared without use of an intermediate subbing layer, by applying directly to the face of an extruded 0.003 inch thick film support of the same poly(hydroxyether) as used in Example 1 a photosensitive emulsion prepared as in Example 2 but containing 20% tetrahydrofuran. After drying the photographic film was exposed to light through a negative. After developing, fixing and washing by the technique of Example 2 a clear reverse image of the negative was obtained. The film support coating adhered tenaciously to the film support throughout developing. No curling occurred.

### EXAMPLE 4

A photographic film was prepared without use of an intermediate subbing layer by applying directly to the face of an extruded 0.003 inch thick film support of the same poly(hydroxyether) as used in Example 1, a photosensitive emulsion prepared as in Example 2 but which contained a total of 1500 cc. water.

To this emulsion was added 30% tetrahydrofuran. Film supports were coated with this mixture at coating thicknesses of from 0.0003 inch to 0.001 inch. Exposure and development were carried out as in Example 2. All coatings gave good images after exposure to light through negatives. All coatings adhered firmly to the film support during developing.

**Control 4A.**—The photosensitive emulsion used in Example 4 was solvent modified as in Example 4 but with 22% acetone in place of the 30% tetrahydrofuran in an attempt to obtain good bonding of the emulsion directly to cellulose triacetate. Photosensitive coatings 0.0003 inch thick and thicker were applied to cellulose triacetate film support. After exposure the films were developed as in Example 4. Immersion in the developer solution lifted each of the photosensitive coatings from the cellulose triacetate film support.

**Control 4B.**—The photosensitive emulsion used in Example 4 was solvent modified as in Example 4 but with 17.8% dioxane in place of the 30% tetrahydrofuran in an attempt to obtain good bonding of the emulsion directly to polycarbonate. Photosensitive coatings 0.003 inch thick and thicker were applied to polycarbonate film support. The coatings were streaked and appeared not to wet the polycarbonate film support. After exposure the films were developed as in Example 4. Immersion in the developer solution lifted each of the photosensitive coatings from the polycarbonate film support.

### EXAMPLE 5

A photographic film was prepared using a 0.001 inch thick film support cast onto a glass plate from a 25% solution in tetrahydrofuran of a poly(hydroxyether) having a reduced viscosity of 0.49 measured as above and the recurring unit



The cast film was air dried at 68° F. and 50% relative humidity for 24 hours and at 110° F. for an additional 24 hours.

A subbing having the formulation given in Example 2 was applied by brush to the face of the cast film support and allowed to air dry. A photosensitive emulsion prepared in darkness using

|    |                                                |      |      |
|----|------------------------------------------------|------|------|
| 5  | (1) Mixed silver halides (dehydrated emulsion) | g--  | 75   |
|    | Dissolved in water                             | cc-- | 750  |
| 10 | (2) Saponin                                    | g--  | 1.5  |
|    | Dissolved in water                             | cc-- | 98.5 |
| 15 | (3) Methanol                                   | cc-- | 50   |
|    | (4) Ammonium chrome alum                       | g--  | 0.5  |
|    | Dissolved in water                             | cc-- | 5    |

was applied in a thin coating with a sponge to the subbing layer on the film support. A uniform and smooth coating was obtained.

The photographic film was exposed to light as in the previous examples. Development was carried out as in Example 2. Adhesion of the gelatin and emulsion to the film support was good throughout developing. An excellent transparency was produced with no evidence of curling.

### EXAMPLE 6

A photographic film was prepared without use of a subbing layer by applying directly to the face of a 0.001 inch thick cast film support of the same poly(hydroxyether) as used in Example 5, a mixture of a photosensitive emulsion prepared as in Example 5 and a solvent, tetrahydrofuran, in a ratio 7 parts of the emulsion per 3 parts of the solvent.

The poly(hydroxyether) film support was coated with the solvent modified photosensitive emulsion using a sponge as the applicator, care being taken to wet all spots of the film support. The coating was smooth. The photographic film was exposed to light and developed as in the previous examples. Adhesion of the emulsion to the film support was good throughout developing. An excellent transparency was obtained.

### EXAMPLE 7

A photographic film was prepared using a 0.001 inch thick film support cast onto a glass plate from a 25% solution in tetrahydrofuran of a poly(hydroxyether) having a reduced viscosity of 0.44 measured as above and the recurring unit



The cast film was air dried at 68° F. and 50% relative humidity for 24 hours and at 110° F. for an additional 24 hours.

A subbing having the formulation given in Example 2 was applied by brush to the face of the cast film support and allowed to air dry. A photosensitive emulsion prepared as in Example 5 was applied as a thin coating with a sponge to the subbing layer on the film support. A uniform and smooth coating was obtained.

The photographic film was exposed to light and developed as in the previous examples. Adhesion of the gelatin layer and the photosensitive emulsion layer to the film support was good throughout developing. A clear transparency having a good contrasting image was obtained. No curling occurred.

### EXAMPLE 8

A photographic film was prepared without use of a subbing coat by applying directly to the face of a 0.001 inch thick cast film support of the same poly(hydroxyether) as used in Example 7, a mixture of a photographic emulsion prepared as in Example 5 and a solvent, tetra-

hydrofuran, in a ratio of 7 parts of the emulsion per 3 parts of the solvent.

The poly(hydroxyether) film support was coated with the solvent modified photosensitive emulsion using a sponge as the applicator. The coating was smooth and uniform over most of the film support. The photographic film was exposed to light and developed as in the previous examples. Adhesion of the photosensitive emulsion to the wetted film support was good throughout developing. An excellent transparency was obtained.

### EXAMPLE 9

A photographic film was prepared using a 0.001 inch thick film support cast onto a glass plate from a 25% solution in tetrahydrofuran of a poly(hydroxyether) copolymer. The copolymer was prepared by mixing 57 grams (0.25 mole) of 2,2-bis(p-hydroxyphenol)-propane and 74.1 grams (0.25 mole) of bisphenol of vinylcyclohexene, 46.3 grams of epichlorohydrin and 106.8 grams of ethyl alcohol together, and after the reaction mixture had been stirred for 15 minutes, adding 22 grams of sodium hydroxide in 69.7 grams of water and then heating the mixture at reflux for five hours. The copolymer had a reduced viscosity of 0.54 measured as above.

The cast film was air dried at 68° F. and 50% relative humidity for 24 hours and at 110° F. for an additional 24 hours. A subbing having the formulation given in Example 2 was applied by brush to the face of the cast film support and allowed to air dry.

A photosensitive emulsion prepared as in Example 5 was applied as a thin coating with a sponge to the subbing layer on the film support. A uniform and smooth coating was obtained.

The photographic film was exposed to light and developed as in the previous examples. Adhesion of the gelatin layer and the photosensitive emulsion was good throughout developing. A transparency with a good contrasting image was obtained. No curling occurred.

### EXAMPLE 10

A photographic film was prepared by applying directly to the face of a 0.001 inch thick cast film support of the same poly(hydroxyether) copolymer as used in Example 9, a mixture of a photographic emulsion prepared as in Example 5 and a solvent, tetrahydrofuran, in a ratio of 7 parts of the emulsion per 3 parts of the solvent.

The poly(hydroxyether) film support was coated with the solvent modified photosensitive emulsion using a sponge as the applicator. A smooth and uniform coating was obtained over a major portion of the film support. The photographic film was exposed to light and developed as in the previous examples. Adhesion of the photosensitive emulsion to the wetted film support and the image produced were excellent. No curling occurred.

What is claimed is:

1. A dimensionally stable and curl-free photosensitive film comprising a film support of a thermoplastic poly(hydroxyether) containing recurring units having the formula



wherein E is the nucleus of a dihydric polynuclear phenol in which the hydroxyl groups are attached to different nuclei and R and R' are each selected from hydrogen and methyl and having a reduced viscosity of from 0.3 to 1.2 measured as a 0.2 gram sample in 100 millimeters of tetrahydrofuran at 25° C. and an image producing photosensitive layer adhered to said film support.

2. A dimensionally stable and curl-free photographic film comprising a film support of a thermoplastic poly-

10 12 (hydroxyether) containing recurring units having the formula



15 wherein E is the nucleus of a dihydric polynuclear phenol in which the hydroxyl groups are attached to different nuclei and R and R' are each selected from hydrogen and methyl and having a reduced viscosity of from 0.3 to 1.2 measured as a 0.2 gram sample in 100 milliliters of tetrahydrofuran at 25° C. and an image producing photosensitive gelatin emulsion adhered to said film support.

3. The photographic film claimed in claim 2 wherein the poly(hydroxyether) film support is cast from solution and is from 0.001 to 0.010 inch in thickness.

4. The photographic film claimed in claim 2 wherein the poly(hydroxyether) film support is extruded and is from 0.001 to 0.010 inch in thickness.

5. A dimensionally stable and curl-free photographic film comprising a film support of a thermoplastic poly(hydroxyether) containing recurring units having the formula



25 30 wherein E is the nucleus of a dihydric polynuclear phenol in which the hydroxyl groups are attached to different nuclei and R and R' are each selected from hydrogen and methyl and having a reduced viscosity of from 0.43 to 0.65 measured as a 0.2 gram sample in 100 milliliters of tetrahydrofuran and, adhered to the film support, an image producing photosensitive emulsion containing gelatin, a silver halide and a water soluble solvent for said poly(hydroxyether).

35 40 6. The photographic film claimed in claim 5 wherein the poly(hydroxyether) has the recurring unit



45 50 7. The photographic film claimed in claim 5 wherein the poly(hydroxyether) has the recurring unit



55 60 8. The photographic film claimed in claim 5 wherein the poly(hydroxyether) has the recurring unit



65 70 9. The photographic film claimed in claim 5 wherein the poly(hydroxyether) is a copolymer prepared by the condensation in an alkaline medium of 2,2-bis-(p-hydroxyphenyl) propane and 1,1-bis-(p-hydroxyphenyl)-2-phenylethane with epichlorohydrin.

13

10. A dimensionally stable and curl-free photographic film comprising a film support of a thermoplastic poly(hydroxyether) containing recurring units having the formula



wherein E is the nucleus of a dihydric polynuclear phenol in which the hydroxyl groups are attached to different nuclei and R and R<sup>1</sup> are each selected from hydrogen and methyl and having a reduced viscosity of from 0.43 to 0.65 measured as a 0.2 gram sample in 100 milliliters of tetrahydrofuran at 25° C., a subbing layer containing gelatin adhered to the film support and an image producing photosensitive emulsion containing gelatin and a silver halide adhered to said subbing.

11. The photographic film claimed in claim 10 wherein the poly(hydroxyether) has the recurring unit



14

12. The photographic film claimed in claim 10 wherein the poly(hydroxyether) has the recurring unit



13. The photographic film claimed in claim 10 wherein the poly(hydroxyether) has the recurring unit



14. The photographic film claimed in claim 10 wherein the poly(hydroxyether) is a copolymer prepared by the condensation in an alkaline medium of 2,2-bis-(p-hydroxyphenyl) propane and 1,1-bis-(p-hydroxyphenyl)-2-phenylethane with epichlorohydrin.

No references cited.

NORMAN G. TORCHIN, *Primary Examiner.*